

Jan. 15, 1929.

1,699,205

E. PODSZUS ET AL

PROCESS OF PRODUCING METAL POWDER PARTICLES OF SPHERICAL SHAPE

Filed July 16, 1926

Fig. 1.



Fig. 2.



Fig. 3.



Fig. 4.



Fig. 5.



Inventors:

Emil Podszus  
and Marvin Kramer  
By Alfred M. \_\_\_\_\_

Atty.

## UNITED STATES PATENT OFFICE.

EMIL PODSZUS, OF BERLIN-FRIEDRICHSHAGEN, AND ERWIN KRAMER, OF BERLIN, GERMANY, ASSIGNEES TO HARTSTOFF-METALL AKTIENGESELLSCHAFT (HAME-TAG), OF BERLIN-COPENICK, GERMANY.

## PROCESS OF PRODUCING METAL-POWDER PARTICLES OF SPHERICAL SHAPE.

Application filed July 16, 1926, Serial No. 122,786, and in Germany October 10, 1925.

My invention relates to the production of metal powder particles and has for its special object to produce metal powder particles constituting hollow spheres.

5. By means of this invention it is possible to produce metal powder whose particles measure about  $\frac{1}{2}$  mm. to 1/100 mm. and less, and such powder can be made from the most heterogeneous kinds of metal and even 10 from ingot-iron of great strength.

Metal powders of this kind are required for the manufacture of pressed bodies, as for example dynamo brushes, sliding contact members and the like which are made 15 from a mixture of graphite and metal powder, or for magnet cores of induction coils and the like that consists of a mixture of metal powder and insulating substance. The powders used hitherto for these purposes 20 consisted of metal flakes of more or less irregular shapes. A powder in accordance with the present invention, as compared with those known powders, has the advantage that the roundness of its particles or 25 grains in itself causes the grains to lie closer together so that smaller pressures are required in making pressed bodies from them. A further advantage that accrues from the formations of the grains is that 30 individual grains are in the form of hollow bodies. When this hollow-grain metal powder is used together with graphite for making pressed bodies that are to be used as sliding contact members, the hollows in 35 the metal grains become filled with graphite so that each grain carries its own lubricant. When the pressed bodies are used for bearing bushings the hollows in the grains, so far as they are not filled with graphite, will 40 receive lubricating liquid.

In magnet cores, the hollow metal grains give smaller electrical iron losses than solid grains, even if the grains are squeezed to such an extent that the hollows in them are 45 practically closed. It is thus seen that the novel metal powder offers many advantages in various technical applications.

Another important point is that the novel process described herein constitutes the first 50 means of any kind for producing a metal powder having round or spherical grains of the aforesaid size.

The metal powder in accordance with the present invention is produced from powder

whose grains more or less have the shape of 55 small flakes.

The invention is illustrated in the drawing in which

Figs. 1 to 3 show the steps in which the flakes are converted into spherical hollow 60 grains.

Fig. 4 is a section of a grain rounding device and

Fig. 5 is a section through Fig. 4.

Fig. 1 is a section of a flake-shaped 65 powder. In accordance with the invention, the edges of the grain are turned over so as to form a minute trough- or basin-shaped body or grain (Fig. 2) as this process is continued the outer edges of the grain are 70 rounded more and more, until at last a grain in the shape of a hollow sphere as shown in Fig. 3 is obtained. This treatment of the grain may be continued, until it is squeezed to such an extent that its cavity has the 75 form of slit. It will, however, generally be preferable not to continue the treatment up to this point.

The process of shaping the powder particles as illustrated by Figs. 1 to 3 may be 80 carried out with the aid of various types of machines. A very simple machine that may be used for this purpose is that shown in Figs. 4 and 5. It consists of a casing 2 with a lid 3, a shaft 1, journaled in a wall 85 of the casing and arms 4 and 5 attached to the shaft and having broad ends or flukes 6 and 7. A quantity of flake-shaped metal particles only partly filling the casing 2 is inserted into it through closable openings 90 (not shown) and the shaft 1 carrying the arms 4 and 5 is then revolved at a high speed so as to fling the particles against the inner walls of the casing and cause them to roll against said walls. The particles are 95 also flung against each other. After a while, they will assume the shape indicated in Fig. 2 and then gradually are converted into hollow spheres as shown in Fig. 3. If the process there is continued, the particles 100 are squeezed or compressed still more, so that their cavities are reduced into narrow slits, the powder thereby becoming comparatively heavy.

We claim:—

1. The process of imparting to metal powder particles spherical shape, which consists in gradually turning over the edges

of flake-shaped particles, and by continuing said operation finally converting the particles into hollow spheres.

2. The process of imparting to metal powder particles spherical shape, which consists in gradually turning over the edges of flake-shaped particles, and finally bend-

ing them in the same operation into spherical shapes.

In testimony whereof we have affixed our signatures.

**EMIL PODSZUS.**  
**ERWIN KRAMER.**